

## UNITED STATES PATENT OFFICE

2,306,964

## CELLULOSIC FILM

Theodore Rudolph Latour, Kenmore, N. Y., assignor to E. I. du Pont de Nemours & Company, Wilmington, Del., a corporation of Delaware

No Drawing. Application October 3, 1939,  
Serial No. 297,665

18 Claims. (Cl. 106—178)

This invention relates to the stripping of dry cast films, especially continuous webs, from the casting surface. More particularly it appertains to the incorporation of alkyl amine salts of fatty acids in organic solvent soluble cellulose substitution derivative film for facilitating separation of the cast film from the casting wheel.

It is a well known fact that organic solvent soluble cellulose derivatives (substituted celluloses) which have been applied in solution to the surface of such materials as wood, metals, ceramics, plastics and the like, and the solvent evaporated, possess considerable adhesion therefor. When applied for protection purposes the adhesion between the cellulose substituted derivative and the base material upon which it has been coated is a desirable property. This inherent adhesion is very undesirable when the base is employed only as a temporary support during the solvent removal as in the casting of self-supporting film such as sheet wrapping material. It is, in fact, one of the most serious obstacles to the production of satisfactory film.

The conventional details of dry casting continuous films of organic solvent soluble cellulose substitution derivatives are disclosed in U. S. A. Patent No. 1,458,592 (Olson). In general such procedures involve the laying of a film of dope (solution of the cellulose derivative) on to a rotating casting wheel mounted and arranged for the removal of the solvent from the dope during its rotation. The means for the solvent removal may include heating the surface of the wheel or surfaces adjacent thereto, together with devices such as fans for carrying the solvent away from the film. Ordinarily the speed of the wheel and the degree of heating are adjusted so that the desired amount of solvent is removed in somewhat less than one revolution of the casting wheel. Nickel, chromium, stainless steel and other metals and alloys are generally used for surfaces of the casting wheels.

In the continuous casting operation the adhesion between the partially dried film and the casting surface is a frequent source of trouble. It causes the film to break or tear at the place where the film is being stripped from the wheel. This action is especially troublesome at the edges of the film. Even when the film does not tear or break distortion and deformation are quite common due to the high tension required for pulling the film away from the casting surface.

A group of materials has now been discovered which greatly decreases the adhesion between such partially dried film and the metal casting

surface. With the preferred members of the group the adhesion is reduced to such an extent that only a very slight tension is required to strip the film from the casting surface.

This invention had for an object the manufacture of transparent, strong and flexible sheets or films which were undeformed and/or undistorted and/or unmarred and the production of compositions of matter suitable for the casting thereof. A further object was to dry cast toluene-ethanol (80:20) soluble ethyl cellulose into thin, strong, smooth, flexible sheets capable of being easily stripped from the casting wheel while retaining 5% to 15% of the solvent of the casting dope. Further objects were to devise a means of decreasing the adhesion between a dry cast, organic solvent soluble, organic cellulose derivative and the casting surface, to facilitate the removal of partially dried, dry cast, organic cellulose derivatives from casting wheels and belts, and to find materials which could be added to a dry casting solution to make removal of the film easy when only a small proportion of the solvent remains. A general advance in the art and other objects which will appear hereinafter are also contemplated.

It has now been discovered that the alkyl (including hydroxyalkyl and aralkyl) salts of fatty acids containing more than 6 carbon atoms may be incorporated in casting dopes with the result that the film formed therefrom can be easily and satisfactorily removed from the casting surface.

From the following description and specific examples in which are disclosed certain embodiments of the invention as well as details of what is believed to be the best mode for carrying out the invention, it will be apparent how the foregoing objects and related ends are accomplished. The parts are given by weight throughout the application.

## Example I

To a solution containing 15% benzyl cellulose together with 15% (on the basis of the benzyl cellulose) dibutyl phthalate as plasticizer dissolved in a solvent mixture consisting of 80% toluene and 20% ethanol, 2% (on the basis of the benzyl cellulose present) triethanolamine stearate was added. Film was cast from this solution on to a nickel surface and dried. It possessed only a slight adhesion to the nickel surface when compared to a film cast from a similar benzyl cellulose solution to which no triethanolamine stearate had been added.

*Example II*

To a solution containing 15% ethyl cellulose together with 15% (on the basis of the ethyl cellulose) diamyl phthalate as plasticizer dissolved in a solvent mixture consisting of 80% toluene and 20% ethanol, 2% (on the basis of the ethyl cellulose present) benzyl trimethyl ammonium laurate was added. Film was cast from this solution on to a nickel surface and dried. It possessed only a slight adhesion to the nickel surface when compared to a film cast from a similar ethyl cellulose solution to which no benzyl trimethyl ammonium laurate had been added.

*Example III*

To a solution containing 15% ethyl cellulose together with 15% (on the basis of the ethyl cellulose) tributyl phosphate as plasticizer dissolved in a solvent mixture consisting of 80% ethylene dichloride and 20% methanol, 2% (on the basis of the ethyl cellulose present) diethanolamine oleate was added. Film was cast from this solution on to a nickel surface and dried. It possessed only a slight adhesion to the nickel surface when compared to a film cast from a similar ethyl cellulose solution to which no diethanolamine oleate had been added.

*Example IV*

To a solution containing 15% ethyl cellulose together with 15% (on the basis of the ethyl cellulose) triethylene glycol dihexoate as plasticizer dissolved in a solvent mixture consisting of 80% toluene and 20% ethanol, 2% (on the basis of the ethyl cellulose present) monoethanolamine oleate was added. Film was cast from this solution on to a nickel surface and dried. It possessed only a slight adhesion to the nickel surface when compared to a film cast from a similar ethyl cellulose solution to which no monoethanolamine oleate had been added.

*Example V*

To a solution containing 15% ethyl cellulose together with 15% (on the basis of the ethyl cellulose) butyl phthalyl butyl glycolate as plasticizer dissolved in a solvent mixture consisting of 80% toluene and 20% ethanol, 2% (on the basis of the ethyl cellulose present) benzyl trimethyl ammonium myristate was added. Film was cast from this solution on to a nickel surface and dried. It possessed only a slight adhesion to the nickel surface when compared to a film cast from a similar ethyl cellulose solution to which no benzyl trimethyl ammonium myristate had been added.

*Example VI*

To a solution containing 15% benzyl cellulose together with 15% (on the basis of the benzyl cellulose) dibutyl phthalate as plasticizer dissolved in a solvent mixture consisting of 80% toluene and 20% ethanol, 2% (on the basis of the benzyl cellulose present) benzyl trimethyl ammonium palmitate was added. Film was cast from this solution on to a nickel surface and dried. It possessed only a slight adhesion to the nickel surface when compared to a film cast from a similar benzyl cellulose solution to which no benzyl trimethyl ammonium palmitate had been added.

*Example VII*

To a solution containing 15% propyl cellulose together with 15% (on the basis of the propyl

cellulose) diamyl phthalate as plasticizer dissolved in a solvent mixture consisting of toluene-ethanol 80:20, 2% (on the basis of the propyl cellulose present) benzyl trimethyl ammonium myristate was added. Film was cast from this solution on to a nickel surface and dried. It possessed only a slight adhesion to the nickel surface when compared to a film cast from a similar propyl cellulose solution to which no benzyl trimethyl ammonium myristate had been added.

*Example VIII*

To a solution containing 15% ethyl benzyl cellulose together with 15% (on the basis of the ethyl benzyl cellulose) dibutyl phthalate as plasticizer dissolved in a solvent consisting of dioxane, 2% (on the basis of the ethyl benzyl cellulose present) benzyl trimethyl ammonium laurate was added. Film was cast from this solution on to a nickel surface and dried. It possessed only a slight adhesion to the nickel surface when compared to a film cast from a similar ethyl benzyl cellulose solution to which no benzyl trimethyl ammonium laurate had been added.

The dope or cellulose derivative solution containing the strip agents of the invention may be handled and cast in the same manner as the dopes previously known to the art.

The most marked decrease in adhesion between the film and the casting wheel surface had been noted when the casting surface was nickel.

In the preferred mode of operation the film is stripped from the casting wheel while it still contains 5% to 15% of the solvent.

This invention is not limited to the ethyl cellulose of the specific examples although it peculiarly appertains thereto. In general it is, with considerable efficacy, applicable to all kinds of organic derivatives of cellulose which are soluble in organic liquids (solvents), including cellulose esters such as cellulose acetate, cellulose propionate, cellulose butyrate, and the like; mixed esters, such as cellulose aceto-propionate, cellulose aceto-butyrate and the like; cellulose ethers, such as methyl cellulose, ethyl cellulose, propyl cellulose, butyl cellulose, benzyl cellulose and the like; mixed ethers, such as ethyl benzyl cellulose and the like; and mixed cellulose ether esters such as ethyl cellulose acetate, and the like.

The alkyl amine salts of fatty acids comprehended by the present invention are those of fatty acids containing at least 7 carbon atoms. Preferably the fatty acids contain 12 to 20 carbon atoms or more. Especially suitable for the purposes of the present invention are the benzyl trimethyl ammonium salts of lauric, myristic, palmitic, oleic and stearic acids. The results obtained with the triethanolamine, diethanolamine and monoethanolamine salts of the aforementioned acids are also outstanding.

In the preferred embodiments of the invention the alkyl amine salt of the fatty acid is present in amount within the range of 0.5% to 5% by weight on the basis of the cellulose derivative. Higher concentrations are not excluded and may be used in order to secure specific results.

The alkyl amine salts of fatty acids may be used singly or in any combination, and it is to be understood that the invention is not limited to the specific alkyl amine salts listed above or in the specific examples.

The stripping agents of this invention may be

incorporated in the casting dope in any desired manner. If preferred they may be predissolved and the solvent used for dissolving the cellulose derivative. Ordinarily they are incorporated into the solvent simultaneously with the cellulose derivative. In some instances it has been found convenient to add the stripping agent to the solution of the cellulose derivative.

Many of the advantages of the present invention will be apparent from the preceding portion of the specification. Specific mention may be made of the fact that by this invention it is possible to easily and satisfactorily remove the partially dried, dry cast film from a metal or alloy casting wheel at elevated temperatures, and that all danger of tearing or deforming the dry cast film at the stripping point (or line) due to the pull required to separate the film from the casting surface has been removed. The advantage of incorporating in a casting solution a material which decreases the adhesion between the film cast therefrom and the casting surface without undesirably affecting the transparency and surface characteristics of the film will be obvious to those skilled in the art.

I claim:

1. A plasticized, organic solvent soluble, cellulose substitution derivative film containing 0.5% to 5% of benzyl trimethyl ammonium laurate.
2. A film of ethyl cellulose containing 0.5% to 5% of benzyl trimethyl ammonium salt of fatty acid containing at least 7 carbon atoms.
3. The product of claim 2 when the fatty acid contains 12 to 20 carbon atoms.
4. A film of ethyl cellulose containing 0.5% to 5% of benzyl trimethyl ammonium salt of acid material from the group consisting of lauric acid, myristic acid, palmitic acid, maleic acid and stearic acid.
5. A film of ethyl cellulose containing 0.5% to 5% of benzyl trimethyl ammonium laurate.
6. A casting dope comprising essentially a 15% solution of ethyl cellulose in organic solvent containing 15% (based on the ethyl cellulose) plasticizer and 2% (based on the ethyl cellulose) benzyl trimethyl ammonium laurate.
7. A casting dope comprising essentially a 15% solution of ethyl cellulose in an 80:20 mixture of toluene-ethanol containing 15% (based on the ethyl cellulose) diamyl phthalate and 2% (based on the ethyl cellulose) benzyl trimethyl ammonium laurate.
8. A casting dope comprising essentially a 15% solution of ethyl cellulose in organic solvent containing 15% (based on the ethyl cellulose) plasticizer and 2% (based on the ethyl cellulose) benzyl trimethyl ammonium myristate.
9. A casting dope comprising essentially a 15%

solution of ethyl cellulose in an 80:20 mixture of toluene-ethanol containing 15% (based on the ethyl cellulose) butyl phthalyl butyl glycolate and 2% (based on the ethyl cellulose) benzyl trimethyl ammonium myristate.

5. 10. A casting dope comprising essentially a 15% solution of ethyl cellulose in organic solvent containing 15% (based on the ethyl cellulose) plasticizer and 2% (based on the ethyl cellulose) benzyl trimethyl ammonium palmitate.
10. 15. A casting dope comprising essentially a 15% solution of ethyl cellulose in an 80:20 mixture of toluene-ethanol containing 15% (based on the ethyl cellulose) dibutyl phthalate and 2% (based on the ethyl cellulose) benzyl trimethyl ammonium palmitate.
15. 20. A casting dope comprising essentially a 15% solution of ethyl cellulose in organic solvent containing 15% (based on the ethyl cellulose) plasticizer and 2% (based on the ethyl cellulose) benzyl trimethyl ammonium salt of fatty acid containing at least 7 carbon atoms.
20. 25. 13. A plasticized organic solvent soluble cellulose substitution derivative film containing 0.5% to 5% of benzyl trimethyl ammonium salt of fatty acid containing at least 7 carbon atoms and 5% to 15% organic solvent for the cellulose substitution derivative.
25. 30. 14. A plasticized organic solvent soluble cellulose substitution derivative film containing 0.5% to 5% of benzyl trimethyl ammonium laurate and 5% to 15% residual casting solvent consisting of an 80:20 toluene-ethanol mixture.
30. 35. 15. A plasticized organic solvent soluble cellulose substitution derivative film containing 0.5% to 5% of benzyl trimethyl ammonium salt of fatty acid from the group consisting of lauric acid, myristic acid, palmitic acid and stearic acid and 5% to 15% organic solvent for the cellulose substitution derivative.
35. 40. 16. A plasticized organic solvent soluble cellulose substitution derivative film containing 0.5% to 5% of benzyl trimethyl ammonium salt of fatty acid containing at least 7 carbon atoms.
40. 45. 17. A casting dope comprising essentially a 15% solution of organic solvent soluble cellulose substitution derivative in organic solvent containing 15% (based on the cellulose derivative) plasticizer and 2% (based on the cellulose derivative) benzyl trimethyl ammonium salt of fatty acid containing at least 7 carbon atoms.
45. 50. 18. A plasticized organic solvent soluble ethyl cellulose film containing 0.5% to 5% of benzyl trimethyl ammonium laurate and 5% to 15% residual casting solvent consisting of an 80:20 toluene-ethanol mixture.

THEODORE R. LATOUR.